

Dec. 19, 1933.

P. L. J. MIGUET

1,939,913

PROCESS FOR ELECTROTHERMIC REDUCTION

Filed July 3, 1930

**FIG.1**



**FIG.2**



**FIG.3**



*Witnesses*

*Henri Germaine  
Jean Maureau*

*Inventor*

*Paul Louis Joseph Miguet  
Blingey, Atto.*

## UNITED STATES PATENT OFFICE

1,939,913

PROCESS FOR ELECTROTHERMIC  
REDUCTIONPaul Louis Joseph Miguet, St.-Julien-de-  
Maurienne, FranceApplication July 3, 1930, Serial No. 465,718,  
and in France November 4, 1925

5 Claims. (Cl. 75—22.5)

This invention relates to an improved process for reducing materials in an electric furnace. This application is in part a continuation of my co-pending application Serial No. 121,189, filed July 8, 1926.

According to the known prior processes of feeding electric furnaces having a vertical electrode, the materials of the charge have been intimately mixed and the proportions of these materials have been only changed to correct the defects which result from the incorrect proportions. This method of charging furnaces results in local overheating of the electrode especially at the end of the electrode. Such overheating causes a loss of about 20% in the raw materials and a loss of about 50% in the energy input. These losses are primarily due to a concentration of the current at the end of the electrode which causes an excessive overheating at this point. The high temperatures there give rise to an excessive formation of gas, which rapidly escapes through the charge around the electrode, thereby causing excessive heating and decomposition of the electrode and loss of heat, and of raw materials.

According to applicant's invention, the raw materials of the furnace charge are divided into conductive and non-conductive batches. These batches are fed separately into the furnace chamber so that they form alternate substantially horizontal layers of conductive and non-conductive material around the vertical electrode. The conductive layers of raw materials extend from the electrode to the conductive portion of the furnace and the non-conductive layers may extend from the vertical electrode towards the furnace walls for only a portion of the distance which separates these elements. This arrangement of the layers of the materials provides a conductive path for the current through the conductive layers and between the non-conductive layers.

In general, the conductive batch may be composed of a mixture of carbonaceous material and an ore to which mixture a flux may or may not be added and the non-conductive batch may be composed of a flux with which a portion of the ore may or may not be mixed as desired. The proportions of the materials in the conductive batch may be changed within certain limits to give the proper conductivity to the conductive layers of material and to provide the correct quantities of reducing agents to react most favorable with the ores. Thus, by changing the proportions of conductive materials to the non-conductive materials in the conductive layer of the

furnace charge, the density of the current in the layer, the spreading of the current and the size of the reducing zone can be increased or decreased within a wide range to produce a most satisfactory condition for each product. These changes of proportions in the conductive layers may be made either by altering the proportion of carbonaceous material to the ore in the furnace charge, or by changing the distribution of the ore or flux, or both, between the conductive and non-conductive batches.

Specific examples of the proportions of the materials contained in the batches will be given infra.

It is preferable to use a very large electrode which carries high current at a low voltage and low density. The low voltage and low density of current aids in the spreading action of the current due to the decreased tendency of the current to form arcs and thereby open up individual conductive paths through the charge. By the use of a large electrode, an interval of space can be maintained more easily between the end of the electrode and the molten baths. This space resists the passage of the current from the end of the electrode to the materials or molten bath thereunder and further aids in the spread of the current laterally from the sides of the electrode. Also by the use of the large electrode the bath is better protected from the falling of the raw materials, in the unreduced state, into the bath and thereby contaminating it. It is stated as an example only, to which I do not wish to be specifically limited, that I have used electrodes varying in amperage from 50,000 to 300,000 amperes with a current density of about 2 amperes per sq. cm.

One of the objects of my invention is to increase the zone of reduction and to cause a lateral reduction of the materials as they pass downward along the electrode and to complete the reduction of these materials before they reach the molten bath.

Another object of my invention is to more effectively control the temperatures of reaction and thereby prevent the excessive formation of gases and reciprocal reactions and heat losses incident thereto.

Another object of my invention is to eliminate local overheating of the electrode and the charge.

Another object of my invention is to increase the life of the electrode.

Another object of my invention is to reduce the ores and refine the final product simultaneously.

Another object of my invention is to produce alloys directly from the ores.

Another object of my invention is to improve the final product.

5 Another object of my invention is to increase the production of the final product per unit of electrical energy used.

Another object of my invention is to suppress the white flames which tend to rise around the 10 electrode at the top of the charge.

The process of my invention is more fully disclosed in the following description, and accompanying drawing in which similar parts in the different figures are referred to by the same letters, and in which:

Figure 1 is a vertical section of an electric furnace having a homogeneous charge fed therein according to the prior known methods.

Figure 2 is a vertical section of an electric furnace showing alternate layers of conductive and non-conductive materials which are fed in accordance with applicant's invention.

20 Figure 3 is a vertical section of an electric furnace similar to Fig. 2 but having a central lining 25 of a neutral non-conductive material and having a peripheral lining of conductive materials.

In Fig. 1 is shown the path of the current *a* flowing through the homogeneous charge *b*, which is made uniformly conductive and is fed 30 into a furnace which is operated in accordance with the prior known methods. It will be noted that the current *a* passes from the end of the electrode *c* to the conductive hearth *d* in a very restricted path. Due to the furnace charge being 35 at a higher temperature under the electrode *c* than it is elsewhere, this portion *e* of the charge, including the molten bath, is made more conductive than the remaining portion of the charge and consequently the current *a* will normally 40 follow the path as indicated unless the distance to the sides of the furnace is materially less than the distance to the bottom or unless other abnormal conditions are introduced.

The electrical power is very poorly utilized 45 when it passes in a more or less straight line from the end of the electrode to the hearth *d* directly underneath it. The flow of the current through this zone furnishes heat where it is least needed and causes an excessive temperature 50 to be maintained at this point. Such conditions cause a loss of heat and a volatilization of raw materials which slide under the electrode. Aside from the loss of heat and materials due to 55 the excessive volatilization of the materials, the carbon monoxide formed thereby causes a very bad condition around the furnace for the workmen.

Fig. 2 illustrates the method of feeding the raw 60 materials into the furnace chamber in accordance with my process. It will be seen that the current *a* spreads out laterally through the furnace charge and traverses the entire charge before it reaches the hearth *d*. The current passes 65 through the conductive layers *h* and between the non-conductive layers *f*. An interval or space *t* is provided between the end of the electrode and the molten bath. The resistance resulting from 70 this space in conjunction with the low voltage and the conductive layers which are interposed between non-conductive layers *c* causes the current to spread out laterally through the conductive layers and flow toward carbon hearth *d* and walls *g* of the furnace to complete the electrical circuit only after it has passed through the entire conductive mixture *h*.

In Fig. 3 is another example of my process in which a larger electrode *c* is used than that used in the furnace illustrated, in Fig. 2. In this case the hearth of the furnace comprises an inner central non-conductive or neutral lining *j* surrounded by another peripheral portion *i* made of carbonaceous material. The non-conductive lining *j* offers a resistance to the passage of the current *a* from the end of the electrode *c* through the slag *k* and final product *l*. This resistance alone and also in combination with the resistance offered by the space *t* will act to cause the current to spread out laterally from the electrode and flow through the conductive mixture instead of flowing from the end of the electrode and through the molten bath where the heat produced by the flow of current is least required.

It will be noted that in Figs. 2 and 3 the non-carbonaceous, non-conductive layers *f* are fed in continuous rings around the electrode and that one of these layers is maintained on top of the charge which acts to suppress the white flames which tend to rise around the electrode at this point.

100 It has been stated that the proportion of carbonaceous material in the conductive mixture and the thickness of the non-conductive layers as compared to the thickness of the conductive layers could be changed as may be required. By such regulation and by the use of the resist- 105 ant space *t* at the end of the electrode, which may be used with or without the resistant central lining *j* in the furnace hearth, the current may be so dispersed through the charge that practically no current will flow from the end of 110 the electrode through the molten bath. The heating action of the current in passing laterally through the charge will cause a complete reduction of the raw materials between the sides of the electrode and the side walls of the furnace 115 before these materials can reach the bottom of the furnace hearth.

Final products such as metals and their alloys 120 may be further refined under the electrode. Sufficient heat may be derived for this purpose from the surrounding charge, the end of the electrode and by the passage of additional current from the end of the electrode through the final product. The necessary fluxing or oxidizing 125 materials as may be required for further refining the final product may be provided in the slag on the top of the molten bath. This may be done by increasing the thickness of the non-conductive layer, which contains the flux or basic material, so that some of this may reach 130 the molten bath in a basic state, or additional basic material may be added directly to the bath. Also, alloys may be formed by adding metals of another kind to the bath.

In order to conserve the energy input and 135 raw materials and to utilize to the best advantage the reducing and oxidizing materials added to the ores, it is recommended to use a large electrode and to maintain a thick charge heaped up around the electrode. Such operating con- 140 ditions, however, should be varied in accordance with the type of ores that are being worked and the final product that is to be produced. Higher power can be used on the large electrodes and at the same time the current density 145 can be kept low, which contributes towards the spreading of the current, which in turn heats the charge more efficiently. Where the charge is thick it absorbs the heat generated more effectively as the upper layers have the opportunity 150

of absorbing the heat from the gases generated in the lower layers. The gases in rising are thrown out towards the walls of the furnace, due to the baffles formed by the non-conductive layers and the pasty charge which exists around the electrode. These gases preheat the upper strata of the charge and the cooler portion of the charge near the furnace walls, and the carbon monoxide in these gases will reduce the materials in its passage therethrough.

In refining metals and alloys in accordance with my process, the infusible carbides such as may be present in the charge, or are formed in the furnace, are eliminated from the charge before it reaches the stage of the final product. Although it is not known, it is thought that the elimination of these objectionable compounds is due to the thorough and effective oxidizing action of the oxidizing materials in the charge.

In choosing a reducing carbon, it is desirable to select a carbon having a very low apparent density and a relatively high conductivity. Anthracite coal and hard metallurgical coke are eliminated because of their high density and also because of their low chemical reactivity, although their conductivity may be good. Wood charcoal is also excluded because of its low conductivity as well as its high combustibility in the air, although it has an apparent low density. Therefore, practically, it is necessary to utilize almost exclusively gas coke or the like.

In determining the proportions of carbonaceous material to be used in the charge in reference to its conductivity where metal turnings are employed, such metal turnings should be ignored. It is impracticable to give any specific rule for the ratio of carbonaceous material to the remainder of the charge or to that portion of the charge in the conductive batch or mixture. Generally, it may be stated that by volume the ratio of carbon in the conductive mixture to the other materials in this mixture may vary from two to four parts of carbon to one of other materials in the mixture. In the case of iron ore and other ores of the heavy metal class, the minimum amount of carbon within this limit should be used in the conductive mixture because these ores require a small portion of reducing carbon, and, if the carbon in the mixture is increased beyond this minimum, this would require an increase in the thickness of carbon-free, non-conductive layers which would lead to poor furnace operating conditions. When possible and when the thickness of the non-conductive layers is not made too great, it is advantageous to increase the proportion of carbon in the conductive mixture in order to obtain a better spreading of the current by the corresponding increase in the conductiveness of the mixture and maintaining a better separation of the layers. As a further limitation, the raw materials outside of the conductive mixture should not weigh more than twice the weight of the non-carbonaceous materials of the conductive mixture in the case where two additions of the mixture are fed into the furnace every half-hour, and not more than three times in cases where three additions are fed every half-hour.

In the manufacture of such products as calcium carbide, ferro-manganese and compounds of silicon, the best practical results are obtained by distributing the weight of the raw materials, exclusive of the carbon and any metallic turning, equally between the conductive and non-

conductive batches. In large furnaces employing full power it may be desirable to tap the furnace every hour instead of every hour and one-half. For the hourly tapping it is preferable to feed only two additions each half hour, whereas for one and one-half hour tapping it is preferable to feed three additions each half hour.

The following are given as examples of the composition of charges which are used for the manufacture of some of the important electric furnace products:

*First.*—Case of heterogeneous charges with conductive mixtures according to the minimum rule of volumes.

*First example*

Iron: 10,000 kw. at 45 volts with one electrode.  
Production per hourly tap:

$$\frac{10000 \text{ kw. hr.}}{2000 \text{ kw. hr.}} \text{ per metric ton} = 5000 \text{ kg.} \quad 95$$

Corresponding raw materials:

$$\begin{aligned} \text{Coke } 5000 \times 0.32 &= 1600 \text{ kg. or 4000 liters.} \\ \text{Ore } 5000 \times 1.8 &= 9000 \text{ kg. or 5000 liters.} \\ \text{Lime } 5000 \times 0.22 &= 1100 \text{ kg. or 1222 liters.} \end{aligned} \quad 100$$

Volumetric ratio of carbon to all raw materials.

$$\frac{\text{Coke}}{\text{Ore} + \text{Lime}} : \frac{4000}{5000 + 1222} = 0.64 \quad 105$$

Corresponding conductive mixture:

$$\begin{aligned} \text{Coke } 1600 \text{ kg. or 4000 liters.} \\ \text{Ore } 3000 \text{ kg. or 1666 liters.} \\ \text{Lime } 366 \text{ kg. or 407 liters.} \end{aligned} \quad 110$$

Volumetric ratio of carbon to raw materials in conductive mixture:

$$\frac{\text{Coke}}{\text{Ore} + \text{Lime}} : \frac{4000}{1666 + 407} = 1.92 \quad 115$$

Additions each half-hour:

First {Ore: 3000 kg. (Variable according to the slags which ought to be 120  
Lime: 366 kg. gray for normal iron and  
Second {Ore: 3000 kg. blackish for iron half-decarburized.)  
Lime: 366 kg.

*Second example* 125

Ferro-manganese 76-80%—10,000 kw., 45 volts, with one electrode:

Production per hourly tap:

$$\frac{10000 \text{ kw. hr.}}{3400 \text{ kw. hr.}} \text{ per metric ton} = 2941 \text{ kg.}$$

Corresponding raw materials:

$$\begin{aligned} \text{Coke } 2941 \times 0.65 &= 1911 \text{ kg. or 4777 liters.} \\ \text{Ore } 2941 \times 2.1 &= 6176 \text{ kg. or 2470 liters.} \\ \text{Lime } 2941 \times 0.65 &= 1911 \text{ kg. or 2123 liters.} \end{aligned}$$

Volumetric ratio of carbon to all raw materials:

$$\frac{\text{Coke}}{\text{Ore} + \text{Lime}} : \frac{4777}{2470 + 2123} = 1.04$$

Corresponding conductive mixture:

$$\begin{aligned} \text{Coke } 1911 \text{ kg. or 4777 liters.} \\ \text{Ore } 3088 \text{ kg. or 1235 liters.} \\ \text{Lime } 955 \text{ kg. or 1061 liters.} \end{aligned}$$

Volumetric ratio of carbon to raw materials in conductive mixture:

$$\frac{\text{Coke}}{\text{Ore} + \text{Lime}} : \frac{4777}{1235 + 1061} = 2.08$$

|       |                                                                                                                                                                                                                                                                                                                                                          |                      |
|-------|----------------------------------------------------------------------------------------------------------------------------------------------------------------------------------------------------------------------------------------------------------------------------------------------------------------------------------------------------------|----------------------|
|       |                                                                                                                                                                                                                                                                                                                                                          | <i>First example</i> |
|       | Additions each half-hour:                                                                                                                                                                                                                                                                                                                                |                      |
| First | Ore: 1544 kg. (Variable according to the<br>Lime: 477 kg. appearance of the slag.)                                                                                                                                                                                                                                                                       |                      |
| 5     | Second Ore: 1544 kg.<br>Lime: 477 kg.                                                                                                                                                                                                                                                                                                                    |                      |
| 10    | <i>Second.</i> —Case of heterogeneous charges in<br>which the weight of the material to be reduced is<br>distributed equally between the conductive mix-<br>tures and the carbon-free additions.                                                                                                                                                         |                      |
| 15    | <i>First example</i>                                                                                                                                                                                                                                                                                                                                     |                      |
|       | Calcium carbide 285 liters—10,000 kw. at 60<br>volts with one electrode.                                                                                                                                                                                                                                                                                 |                      |
| 15    | Production by hourly taps:                                                                                                                                                                                                                                                                                                                               |                      |
|       | $\frac{10000 \text{ kw. hr.}}{2900 \text{ kw. hr.}} = \text{per metric ton} = 3448 \text{ kg.}$                                                                                                                                                                                                                                                          |                      |
|       | Corresponding raw materials:                                                                                                                                                                                                                                                                                                                             |                      |
| 20    | Coke $3448 \times 0.75 = 2586$ kg. or 6465 liters.<br>Lime $3448 \times 1. = 3448$ kg. or 3831 liters.                                                                                                                                                                                                                                                   |                      |
|       | Volumetric ratio of carbon to all raw materials:                                                                                                                                                                                                                                                                                                         |                      |
| 25    | $\frac{\text{Coke}}{\text{Lime}} : \frac{6465}{3831} = 1.68$                                                                                                                                                                                                                                                                                             |                      |
|       | Corresponding conductive mixture:                                                                                                                                                                                                                                                                                                                        |                      |
|       | Coke 2586 kg. or 6465 liters.<br>Lime 1724 kg. or 1915 liters.                                                                                                                                                                                                                                                                                           |                      |
| 30    | Volumetric ratio of carbon to raw materials in<br>conductive mixture:                                                                                                                                                                                                                                                                                    |                      |
| 35    | $\frac{\text{Coke}}{\text{Lime}} : \frac{6465}{1915} = 3.37$                                                                                                                                                                                                                                                                                             |                      |
|       | Additions each half-hour:                                                                                                                                                                                                                                                                                                                                |                      |
| 40    | First: Lime 862 kg. (Variable according to<br>Second: Lime 862 kg. the appearance of<br>the taps.)                                                                                                                                                                                                                                                       |                      |
|       | <i>Second example</i>                                                                                                                                                                                                                                                                                                                                    |                      |
|       | Ferro-silicon 45%—10,000 kw. at 50 volts, with<br>one electrode.                                                                                                                                                                                                                                                                                         |                      |
|       | Production by hourly taps:                                                                                                                                                                                                                                                                                                                               |                      |
|       | $\frac{10000 \text{ kw. hr.}}{5700 \text{ kw. hr.}} = \text{per metric ton} = 1754 \text{ kg.}$                                                                                                                                                                                                                                                          |                      |
|       | Corresponding raw material:                                                                                                                                                                                                                                                                                                                              |                      |
| 50    | Coke $1754 \times 0.5 = 877$ kg. or 2192 liters.<br>Quartz $1754 \times 1. = 1754$ kg. or 1349 liters.<br>Turnings $1754 \times 0.6 = 1052$ kg. or 2104 liters.                                                                                                                                                                                          |                      |
| 55    | Volumetric ratio of carbon to raw materials<br>(the turnings being ignored):                                                                                                                                                                                                                                                                             |                      |
|       | $\frac{\text{Coke}}{\text{Quartz}} : \frac{2192}{1349} = 1.62$                                                                                                                                                                                                                                                                                           |                      |
|       | Corresponding conductive mixture:                                                                                                                                                                                                                                                                                                                        |                      |
| 60    | Coke 877 kg. or 2192 liters.<br>Quartz 877 kg. or 674 liters.<br>Turnings 1052 kg. or 2104 liters.                                                                                                                                                                                                                                                       |                      |
| 65    | Volumetric ratio of carbon in conductive mix-<br>ture (the turnings being ignored):                                                                                                                                                                                                                                                                      |                      |
|       | $\frac{\text{Coke}}{\text{Quartz}} : \frac{2192}{674} = 3.25$                                                                                                                                                                                                                                                                                            |                      |
|       | Additions each half-hour:                                                                                                                                                                                                                                                                                                                                |                      |
| 70    | First: Quartz 438 kg. (Varied according to<br>Second: Quartz 438 kg. whether slag appears or<br>as tapping is slow.)                                                                                                                                                                                                                                     |                      |
| 75    | <i>Third.</i> —Case of heterogeneous charges with<br>one of the materials to be reduced placed entire-<br>ly in the conductive mixture.                                                                                                                                                                                                                  |                      |
|       | Calcium-silicon—CaSi <sub>3</sub> —10,000 kw. at 50 volts<br>with one electrode.                                                                                                                                                                                                                                                                         |                      |
|       | Production by hourly taps:                                                                                                                                                                                                                                                                                                                               | 80                   |
|       | $\frac{10000 \text{ kw. hr.}}{12000 \text{ kw. hr.}} = \text{per metric ton} = 833 \text{ kg.}$                                                                                                                                                                                                                                                          |                      |
|       | Corresponding raw materials:                                                                                                                                                                                                                                                                                                                             |                      |
|       | Coke 833 $\times 0.89 = 741$ kg. or 1852 liters.<br>Lime 833 $\times 0.52 = 433$ kg. or 481 liters.<br>Quartz 833 $\times 1.64 = 1366$ kg. or 1050 liters.                                                                                                                                                                                               | 85                   |
|       | Volumetric ratio of carbon to all raw materials:                                                                                                                                                                                                                                                                                                         |                      |
|       | $\frac{\text{Coke}}{\text{Lime} + \text{Quartz}} : \frac{1852}{481 + 1050} = 1.20$                                                                                                                                                                                                                                                                       |                      |
|       | Corresponding conductive mixture:                                                                                                                                                                                                                                                                                                                        |                      |
|       | Coke 741 kg. or 1852 liters.<br>Lime 433 kg. or 481 liters.                                                                                                                                                                                                                                                                                              | 95                   |
|       | Volumetric ratio of carbon to the raw mate-<br>rials in the conductive mixture:                                                                                                                                                                                                                                                                          |                      |
|       | $\frac{\text{Coke}}{\text{Lime}} : \frac{1852}{481} = 3.85$                                                                                                                                                                                                                                                                                              | 100                  |
|       | Additions each half-hour:                                                                                                                                                                                                                                                                                                                                |                      |
|       | First: Quartz 683 kg. (Varied according to wheth-<br>Second: Quartz 683. er slag appears or as tap-<br>ping is slow.)                                                                                                                                                                                                                                    | 105                  |
|       | <i>Second example</i>                                                                                                                                                                                                                                                                                                                                    |                      |
|       | Calcium - aluminum - silicon—CaAlSi <sub>2</sub> —15,000<br>kw. at 50 volts with one electrode.                                                                                                                                                                                                                                                          |                      |
|       | Production by tapping every one and one-half<br>hours:                                                                                                                                                                                                                                                                                                   | 110                  |
|       | $\frac{15000 \text{ kw. hr.}}{12000 \text{ kw. hr.}} = \text{per metric ton} = 1250 \text{ kg.}$                                                                                                                                                                                                                                                         |                      |
|       | Corresponding raw materials:                                                                                                                                                                                                                                                                                                                             | 115                  |
|       | Coke $1250 \times 0.85 = 1062$ kg. or 2655 liters.<br>Lime $1250 \times 0.53 = 662$ kg. or 735 liters.<br>Quartz $1250 \times 1.1 = 1375$ kg. or 1057 liters.<br>Corundum $1250 \times 0.45 = 562$ kg. or 200 liters.                                                                                                                                    | 120                  |
|       | Volumetric ratio of carbon to all raw materials:                                                                                                                                                                                                                                                                                                         |                      |
|       | $\frac{\text{Coke}}{\text{Lime} + \text{Quartz} + \text{Corundum}} : \frac{2655}{735 + 1057 + 200} = 1.33$                                                                                                                                                                                                                                               |                      |
|       | Corresponding conductive mixture:                                                                                                                                                                                                                                                                                                                        | 125                  |
|       | Coke 1062 kg. or 2655 liters.<br>Lime 662 kg. or 735 liters.                                                                                                                                                                                                                                                                                             |                      |
|       | Volumetric ratio of carbon to raw materials<br>in the conductive mixture:                                                                                                                                                                                                                                                                                | 130                  |
|       | $\frac{\text{Coke}}{\text{Lime}} : \frac{2655}{735} = 3.61$                                                                                                                                                                                                                                                                                              |                      |
|       | Additions each half-hour:                                                                                                                                                                                                                                                                                                                                |                      |
|       | First: Quartz 687 kg. (Varied according as to<br>Second: Corundum 562 kg. whether slag appears<br>Third: Quartz 687 kg. or as tapping is<br>slow.)                                                                                                                                                                                                       | 135                  |
|       | The manufacture of the above indicated prod-<br>ucts is not limited to the exact proportions of the<br>charge as given herein, as these proportions<br>should be varied in accordance with the quality<br>and kind of raw materials used.                                                                                                                | 140                  |
|       | Due to the efficiency of my process described<br>herein, ores of low recovery content may be com-<br>mercially worked which were impracticable to<br>work heretofore. This process is further en-<br>hanced in value by the apparatus described in<br>Patent No. 1,680,163 granted Aug. 7, 1928, on an<br>application filed by me which is a division of |                      |

application Serial No. 121,189 of which this application is a continuation in part. The apparatus referred to discloses an efficient means for separately feeding each batch of materials into the furnace by feeding portions of each addition simultaneously from a number of points about the electrode so that they will be thrown against the electrode.

I claim:

10. 1. The method of operating an electric furnace having a vertical electrode, said method comprising forming the charge in alternate conducting and non-conducting strata, said conductive strata extending from the electrode to the walls of the furnace and said non-conductive strata extending for only a portion of the distance from the electrode to the walls of the furnace, connecting the electrode and a portion of the furnace at the side of the electrode in circuit with a source of power whereby the current is allowed to spread through the conductive strata above the lower end of the electrode thereby heating the charge laterally.
2. The method of operating an electric furnace comprising forming alternate conductive and non-conductive strata of materials which surround the electrode; said conductive strata extending from the electrode to the walls of the furnace and said non-conductive strata extending for only a portion of the distance from the electrode to the walls of the furnace; directing current into the electrode; intercepting the flow of current from the end of the electrode through the molten bath to the hearth by interposing a resistance in such path, and causing said current to spread laterally from the side of the electrode and spread laterally through the conductive strata to the furnace hearth.
3. The method of operating an electric furnace having a vertical electrode and a hearth having at least the outer edges connected to a power circuit, which comprises forming successively alternate conductive and non-conductive strata of material around the electrode, said conductive strata extending from the electrode to the walls of the

furnace and said non-conducting strata extending for only a portion of the distance from the electrode to the walls of the furnace, directing current at the low voltage into the electrode, intercepting the flow of current from the end of the electrode through the molten bath to the hearth by interposing a resistance between the electrode and the conductive portion of the hearth and causing said current to spread laterally from the sides of the electrode through the conductive strata and thence to the conductive portion of the hearth.

4. The method of operating an electric furnace comprising forming successively, alternate conductive and non-conductive strata of material around a large electrode; said conductive strata extending from the electrode to the walls of the furnace and said non-conductive strata extending for only a portion of the distance from the electrode to the walls of the furnace; directing high current at low voltage into the electrode, and causing a current of low density to flow therein; intercepting the flow of current from the end of the electrode through the molten bath to the hearth by interposing an interval of space between the end of the electrode and the materials thereunder; and causing the current to spread laterally through the conductive strata and thereby reduce the charge between the side of the electrode and the furnace wall.

5. The method of operating an electric furnace having a vertical electrode comprising one electric terminal and a hearth having at least a portion thereof conductive and comprising the other electric terminal; said method comprising charging alternate layers of conductive and non-conductive materials into said furnace, so that said conductive layers extend to the walls of said furnace and said non-conductive layers do not extend to the walls of said furnace, whereby the current is carried laterally through the conductive layers from the electrode and downwardly to the furnace hearth.

PAUL LOUIS JOSEPH MIGUET.

45

120

50

125

55

130

60

135

65

140

70

145

75

150